

## UNITED STATES PATENT OFFICE

2,527,379

## SILVER HALIDE DEVELOPERS FOR THE PRODUCTION OF AZINE DYESTUFF IMAGES

Willy A. Schmidt and Robert C. Gunther, Easton, Pa., assignors to General Aniline & Film Corporation, New York, N. Y., a corporation of Delaware

No Drawing. Application July 15, 1948,  
Serial No. 38,948

5 Claims. (Cl. 95—88)

1

The present invention relates to the production of azine dye images and more particularly to color developers designed to yield such images of good gradation and dye density and free from color fog.

In the conventional mechanism of color forming development, an aromatic primary amine is employed to reduce an exposed silver halide image to metallic silver, the amine being thereby oxidized to a component which couples with a color former to produce a dyestuff image in situ with the metallic silver image. To date all color forming development processes which have been commercially exploited have as the developer an N,N-dialkylated-p-phenylene diamine. Such developers have been used for development of a latent image as well as for the development of a residual silver halide image in the reversal process.

Schmidt and Tulagin, in their application Serial No. 640,382, filed January 10, 1946, now Patent No. 2,486,440, disclosed that azine dye images can be obtained by developing an exposed silver halide emulsion with developers of the 2,4-diamino aniline type, and particularly those of the class of the N-substituted 4,6-diamino metanilic acids. The azine dye images which result from this method are much more stable to acids, alkalies and alkaline oxidation than are the azo methine and quinonimine dyes produced with the generally employed p-phenylene diamine type developers.

One of the difficulties which has been encountered in the production of azine dye images by color development resides in the fact that while some 2,4-diamino anilines are capable of developing a latent image, a large number of them are unsatisfactory, yielding either no images at all or only very weak images. It has been proposed to energize such development, particularly when developing a residual silver halide in the reversal process by use with the 2,4-diamino aniline developers of nitrogenous bases, such as ethylenediamine, benzylamine, quinoline, and the like.

We have now ascertained that the formation of azine dye images can be uniformly and energetically effected while obtaining improved color rendition and substantially no color fog by carrying out the development in part with an energetic latent image developer for the exposed silver

2

halide which does not necessarily take part in the color forming reactions, the complete development being effected with one of the aforesaid azine dye forming color developers. The energetic latent image developers contemplated herein are those generally referred to in color photography as silver developers or "black and white" developers.

The partial development effected by the energetic latent image developer may be realized by bathing the exposed silver halide in such a developer for a short period of time and then developing with the 2,4-diamino aniline developer or by adding the energetic developer to the color developer proper.

The particular cooperation which takes place between the energetic latent image developer and the color developer has not been ascertained. It was our original theory that the energetic

latent image developer operated as a catalyst or accelerator for the color developer in the development of a latent image. This theory, however, would not explain the fact that the film can be washed for  $\frac{1}{2}$  hour or longer after an extremely short treatment with the energetic developer and the latent image still be capable of being completely developed by the color developer. It is our opinion, therefore, that the energetic or black and white developer leads to an intensification of the latent image or produces silver nuclei or development centers which aid or facilitate the reduction of additional exposed silver halide by the azine dye forming color developer.

It is accordingly an object of the present invention to produce uniformly and energetically azine dyestuff images with an azine dye forming color developer by carrying out a portion of the development with an energetic latent image developer.

It is a further object of the present invention to improve the azine dye images obtained by color development with an azine dye-forming color developer by adding to the developer an energetic latent image developer.

A further object of the present invention is to produce azine dye images which have improved color rendition and freedom from color fog by developing an exposed silver halide emulsion in the presence of a color former with a 4,6-diamino metanilic acid developer containing an energetic latent image developer.

## 3

Other and further important objects will become apparent as the description proceeds.

Compounds which may be used as the color developer in producing the azine dye images are of the 2,4-diaminoaniline type and are more particularly those having the formula:



wherein R is hydrogen or alkyl, i. e., methyl, ethyl, propyl, butyl, amyl or the like, and R<sub>1</sub> is an aliphatic radical such as alkyl as above, carboxy alkyl such as carboxy methyl, carboxy ethyl and the like, hydroxy alkyl such as hydroxy ethyl, hydroxy propyl and the like, sulfo alkyl such as sulfomethyl, sulfopropyl, sulfobutyl and the like, or an aromatic radical such as aryl, i. e., phenyl, naphthyl and the like, carboxy aryl, i. e., carboxy phenyl, carboxy naphthyl and the like, sulfo aryl, i. e., sulfophenyl, sulfonaphthyl and the like, alkoxy aryl such as methoxy phenyl, methoxy naphthyl, ethoxy phenyl, butyroxy phenyl and the like, alkyl aryl such as toluyl, ethylphenyl, propylphenyl and the like, carboxy alkyl-aryl, such as carboxy methyl phenyl, carboxy ethyl phenyl and the like, carboxy alkoxy aryl, such as carboxy methoxy phenyl, carboxy ethoxy phenyl, hydroxy alkyl aryl such as hydroxy methyl phenyl, hydroxy ethyl phenyl and the like, and hydroxy alkoxy aryl such as hydroxy methoxy phenyl, hydroxy ethoxy phenyl and the like, R<sub>2</sub> is an aromatic or aliphatic radical as illustrated above, and X and Y are hydrogen, alkyl as above, sulfo or carboxy, or together represent the atoms necessary to complete a six-membered isocyclic ring system such as benzo and the like. Preferably the compounds which are utilized are the N-substituted 4,6-diamino metanilic acids, in which case Y is hydrogen, and X is sulfo.

Examples of compounds contemplated by the above formula and found to be satisfactory for the production of the azine dye images are:

1. 5-amino-6,8-bis-(phenylamino)-1-naphthalene sulfonic acid of the formula:



2. 2,4-bis-(phenylamino)-aniline of the formula:



## 4

3. 4 - (phenylamino) - 6 - (N-sulfo methyl-N-phenylamino)-metanilic acid.  
 4. 2,4-bis-(2'-carboxyphenylamino)-aniline.  
 5. 2,4-bis-(3'-carboxyphenylamino)-aniline of the formula:



- 10 6. 2,4- bis - (3'- carboxy- 4' - methoxyphenylamino)-aniline.  
 15 7. 4,6-bis-(phenylamino)-metanilic acid.  
 20 8. 4,6-bis-(4'-methoxy phenylamino)-metanilic acid.  
 25 9. 4 - (2'-methoxy phenylamino)-6- (4'-methoxy phenylamino)-metanilic acid.  
 30 10. 4- (4'-methoxy phenylamino)-6- (phenylamino)-metanilic acid.  
 11. 4,6-bis-(2'-methoxy phenylamino)-meta-  
 nnilic acid.  
 12. 4- (3'- carboxyphenylamino)- 6- (4'- methoxy phenylamino)-metanilic acid of the formula:



- 35 13. 4-(3'-carboxy-4'-methoxy phenylamino)-6-(4'-methoxyphenylamino)-metanilic acid.  
 40 14. 4 - (4' - sulfophenylamino) - 6 - (4' - methoxyphenylamino)-metanilic acid.  
 45 15. 2,4 - bis - (phenylamino) - 5 - amino benzoic acid of the formula:



- 50 55 16. 4 - (4' - methoxyphenylamino) - 6 - (3' - carboxymethylphenylamino)-metanilic acid.  
 60 17. 4 - (4' - sulfophenylamino) - 6 - (3' - carboxymethyl - 4' - methoxyphenylamino) - met- anilic acid of the formula:



- 65 70 18. 4 - (4' - methoxyphenylamino) - 6 - di- methylamino-metanilic acid.  
 75 19. 4 - (4' - sulfophenylamino) - 6 - dimethyl- amino-metanilic acid.  
 20. 4 - (4' - methoxyphenylamino) - 6 - (4' - methylphenylamino)-metanilic acid.

21. 2-sulfo ethylamino-4-(2'-carboxy phenylamino)-aniline of the formula:



22. 4 - phenylamino - 6 - (4' - carboxymethoxy-phenylamino)-metanilic acid.

23. 4 - (4' -  $\beta$  - hydroxyethoxy phenylamino) - 6-methylamino-metanilic acid.

24. 4,6 - bis - (3' - carboxymethoxy phenylamino)-metanilic acid.

25. 4 - ( $\beta$  - hydroxyethylamino) - 6 - phenylamino-metanilic acid.

26. 4,6 - bis - ( $\beta$  - hydroxy ethylamino) - metanilic acid.

27. 4 - ethylamino - 6 - ( $\beta$  - hydroxyethylamino)metanilic acid of the formula:



28. 4 - (carboxymethylamino) - 6 - phenylamino-metanilic acid.

29. 4 - butylamino - 6 - (4' -  $\beta$  - hydroxyethylphenylamino)-metanilic acid.

30. 4 - (4' - carboxymethylphenylamino) - 6 - ethylamino-metanilic acid of the formula:



31. 4 - methylamino - 6 - phenylamino - metanilic acid.

32. 4,6 - bis - (methylamino) - metanilic acid.

33. 4 - phenylamino - 6 - methylamino - metanilic acid.

The aforementioned compounds may be utilized per se as the azine dye image developer or may be used in admixture to insure the production of brilliant dye images as described in Gunther's copending application Serial No. 38,808, filed of even date herewith, entitled: "Production of Azine Dye Images By Means of a Developer Containing Two N-Substituted Diamino Metanilic Acids." Examples of such mixtures are: 4-( $\beta$ -hydroxyethylamino)-6-phenylamino-metanilic acid with 4-methylamino-6-phenylamino-metanilic acid, 4,6-bis-(phenylamino)-metanilic acid with 4,6-bis-(methylamino)-metanilic acid.

The developer components listed above may be prepared by the method described in the aforementioned application Serial No. 640,382 and Gunther application Serial No. 793,532, filed December 23, 1947.

Examples of the energetic latent image or black and white developers which are added to the aforementioned color developers in order to effect the desired more energetic development are p-amino phenol, p-(N-methylamino)-phenol or a mixture thereof with hydroquinone, 2,4-diamino phenol and catechol.

If the invention be practiced by bathing an exposed silver halide emulsion in an energetic or black and white developer followed by complete development in an azine dye color forming developer, the development time with the former will depend on the characteristics of the developer chosen, but should not exceed one-half the time which is necessary to develop the silver image to maximum contrast. In this period, the exposed silver halide is so conditioned that it becomes readily amenable to the production of azine dye images with the aforesaid color developers irrespective of the energy of said developers as measured by their effect on a latent silver halide image.

If the invention be carried out by adding the energetic or black and white developer to the color developer, then the quantity of the former used will in no case exceed the quantity by weight of the active color developer ingredient and will depend first upon the particular energetic or black and white developer employed, and, second, upon the type of processing involved, i. e., whether negative or positive. Generally speaking, the more vigorous the developing substance the smaller the amount required to produce the desired effect. Similarly where the processing is by the reversal method, a smaller quantity is used than where the processing involves negative development. In any case good results are obtained when the concentration of energetic or black and white developer ranges from .5 to 4 grams per liter of developer. Within the aforementioned range an amount of .5 to 1.5 grams per liter of developer of the energetic or black and white developer is sufficient to produce the desired improvement in the reversal process. Where, however, it is desired to produce negative azine dyes, the quantity of the energetic or black and white developer employed generally ranges from 2 to 4 grams per liter. With these quantities, the development of a latent silver halide image in the presence of a suitable color former to produce excellent color rendition and dye density and without color fog formation can be effected in from 10 to 15 minutes.

The color formers employed are those used in the production of color developed images, i. e., those containing aromatic-primary amino, phenolic hydroxyl, or active methylene groups.

Examples of such compounds are:

- 5-sulfo-acetoacetanilide
- 3-stearoylamino-5-sulfo-acetoacetanilide
- 2-benzcarbamyl naphthol-7
- 3,6-disulfo-8-benzsulfonylamino naphthol-1
- 8-benzsulfonyl amino naphthol-1
- 3-sulfo-6-aminonaphthol-1
- 3-sulfo-6-phenylaminonaphthol-1
- 3-sulfo - 6 - (4' - methoxy - phenylamino) - naphthol-1
- 8-hydroxy quinoline
- 3-sulfo-6-oleylamino-naphthol-1
- naphsultam acid
- 3-sulfo-7-phenylaminonaphthol-1
- 1,8-bis-(benzsulfonyl amino) -naphthalene
- 6-bromo-8-hydroxy quinoline
- 6-sulfo-8-hydroxy quinoline
- 2-phenyl-6-bromo-8-hydroxy cinchoninic acid
- 6-bromo-8-hydroxy quinaldine
- 6-stearoylamino-2-(2'-phenyl - 6' - bromo-8'-hydroxy cinchoninoyl) -amino toluene-4-sulfonic acid
- 2-phenyl-6-chloro-8-hydroxy cinchoninoyl octadecyl taurine
- 2-methyl-4,5'-dihydroxy-7,8-benzo-quinoline

7

2-methyl-4,4'-dihydroxy-7,8-benzoquinoline  
2-methyl-4-(4'-N-tetradecyl sulfoacetamido  
aniline)-4'-hydroxy-7,8-benzoquinoline.

The quinolines and benzoquinolines referred to hereinabove are described in copending applications Serial Nos. 793,534 and 793,533, now U. S. Patent No. 2,524,741, of Tulagin and Schmidt and Tulagin and Coles, respectively.

The process utilizing the developer compositions contemplated herein may be effected in various ways. For instance, the color-forming component may be located in the developer. On the other hand, the color former in non-diffusing form may be located in the emulsion. Multi-layer film, each layer containing a non-diffusing color former, may be used and the film developed to the desired subtractive azine dye images in a single color forming development step while utilizing such developer compositions.

The developers, in addition to the components previously mentioned, also contain an alkali such as sodium carbonate, sodium hydroxide, and the like. Preferably the developers will also contain the usual adjuncts such as an alkali metal bromide, i. e., potassium bromide, sodium bromide and the like, and an alkali metal sulfite such as sodium sulfite and the like. In some cases it has also been found that better results are obtained when there is present in the developer a coupling aid in the form of an organic base such as pyridine, quinoline, ethylenediamine and the like.

The following examples will serve to illustrate the invention but it is to be understood that the invention is not restricted thereto.

#### Example I

A photographic silver bromide emulsion containing 6-stearoyl-amino-2-(2'-phenyl-6'-bromo-8'-hydroxy-cinchoninoyl)-amino-toluene-4-sulfonic acid as a non-diffusing color former is exposed, the latent image developed to a negative silver image, re-exposed, and the residual silver halide developed for 10 minutes in a solution of the following composition:

|                                            |       |      |
|--------------------------------------------|-------|------|
| 4-methylamino-6-phenylamino-metanilic acid | grams | 6    |
| 2,4-diamino phenol                         | do    | 1    |
| Sodium sulfite                             | do    | 60   |
| Ethylenediamine                            | cc    | 30   |
| Water                                      | cc    | 1000 |

The film after development is bleached with a ferricyanide bleach and fixed in an acid-hardening hypo solution. There is thus obtained a magenta azine dye image of good gradation in which the whites are perfectly clear.

#### Example II

The procedure is the same as that of Example I excepting that the 2,4-diamino phenol is replaced by 1.5 grams of p-amino phenol per liter of developer.

#### Example III

A bi-pack having a red sensitive silver bromide emulsion containing as the cyan color former a compound of the following constitution:



8

in the bottom layer, and a green sensitive silver bromide emulsion containing as the magenta color former a compound of the following constitution:



in the top layer is exposed, the latent image developed to a negative silver image, re-exposed and the residual silver bromide in both layers developed for 15 minutes in a solution of the following composition:

|                                                              |       |      |
|--------------------------------------------------------------|-------|------|
| 4-( $\beta$ -hydroxyethylamino)-6-phenylamino-metanilic acid | grams | 6    |
| p-(N-methylamino) phenol sulfate                             | do    | 1    |
| Potassium carbonate                                          | do    | 20   |
| Sodium sulfite                                               | do    | 60   |
| Potassium bromide                                            | do    | 10   |
| Ethylenediamine                                              | do    | 5    |
| Water                                                        | cc    | 1000 |

The film after development is processed as in Example I. A colored positive containing magenta and cyan azine dye images showing excellent color rendition and freedom from color fog is thus obtained.

#### Example IV

A photographic silver bromide emulsion is exposed and the latent image developed to a negative silver image. The residual silver halide is re-exposed and developed in a developer of the following composition:

|                                                                            |       |      |
|----------------------------------------------------------------------------|-------|------|
| 4,6-bis-(phenylamino)-metanilic acid                                       | grams | 4    |
| A mixture of hydroquinone and p-(N-monomethylamino)-phenol sulfate (50:50) | grams | 1.5  |
| Sodium carbonate                                                           | do    | 60   |
| Sodium sulfite                                                             | do    | 40   |
| Potassium bromide                                                          | do    | 2.5  |
| Pyridine                                                                   | cc    | 12   |
| 8-hydroxy quinoline                                                        | grams | 3    |
| Water                                                                      | cc    | 1000 |

The film after development is bleached in a ferricyanide bleach and fixed in an acid-hardening hypo solution. A positive magenta azine dye image showing excellent color rendition and no color fog is thus obtained.

#### Example V

The bi-pack referred to in Example III is exposed and developed for 15 minutes in a solution of the following composition:

|                                                              |       |      |
|--------------------------------------------------------------|-------|------|
| 4-( $\beta$ -hydroxyethylamino)-6-phenylamino-metanilic acid | grams | 6    |
| 4-methylamino-6-phenylamino-metanilic acid                   | grams | 3    |
| p-(N-methylamino) phenol sulfate                             | do    | 3    |
| Trisodium phosphate                                          | do    | 40   |
| Sodium sulfite                                               | do    | 40   |
| Potassium bromide                                            | do    | 12.5 |
| Hydroxylamine hydrochloride                                  | do    | 1    |
| Water                                                        | cc    | 1000 |

The film after development is fixed in an acid-hardening hypo solution, bleached in a ferricyanide bleach and again fixed. A negative con-

taining brilliant magenta and cyan azine dye images is thus obtained, the whites being exceedingly clear.

Example VI

A photographic silver halide emulsion layer containing an azine color former in non-diffusing form as given in Example III is exposed. It is given a short development (30 to 90 seconds) in a conventional metol-hydroquinone developer. Thereafter it is thoroughly washed for 15 minutes and the development is continued in an azine color forming developer of the following composition:

|                                                               |       |      |
|---------------------------------------------------------------|-------|------|
| 4-( $\beta$ -hydroxy ethylamino)-6-phenylamino metanilic acid | grams | 6    |
| 4-methylamino-6-phenylamino-metanilic acid                    | grams | 3    |
| Trisodium phosphate                                           | do    | 40   |
| Sodium sulfite                                                | do    | 40   |
| Potassium bromide                                             | do    | 12.5 |
| Hydroxylamine hydrochloride                                   | do    | 1    |
| Water                                                         | cc.   | 1000 |

After development, the film is washed for 10 minutes, fixed, and the silver removed in the conventional manner. There results a negative dye image of good gradation and free from color fog.

We claim:

1. The process of producing within a light sensitive photographic silver halide emulsion layer azine dye images of good color gradation and essentially free from color fog, which comprises developing the exposed silver halide in an energetic non-staining silver image developer for not more than half the time necessary to develop the silver image to maximum contrast and completing the development in the presence of a color former with a color forming developer comprising a compound selected from the class consisting of those of the following formulae:



in which R is selected from the class consisting of hydrogen and alkyl, R<sub>1</sub> is selected from the class consisting of aliphatic and aromatic radicals, R<sub>2</sub> is selected from the class consisting of aromatic radicals, a ring carbon atom of which is directly linked to the nitrogen atom, and aliphatic radicals a carbon atom of which is directly linked to the nitrogen atom, said carbon atom being substituted by at least two hydrogen atoms, X and Y are selected from the

class consisting of hydrogen, alkyl, sulfo and carboxy, and Q represents the atoms necessary to complete a six-membered isocyclic ring system.

2. The process as defined in claim 1 wherein the energetic silver image developer is added to the color forming developer solution in an amount not exceeding the quantity by weight of the color forming developer substance.

3. The process as defined in claim 1 wherein the energetic silver image developer is added to the color forming developer and in an amount ranging from .5 to 4 grams per liter of the developing solution.

4. A photographic developer for the production of azine dye images having high color rendition and free from color fog comprising an aqueous alkaline solution of a non-staining silver image developer and as the color forming developer a compound selected from the class consisting of those of the following formulae:



in which R is selected from the class consisting of hydrogen and alkyl, R<sub>1</sub> is selected from the class consisting of hydrogen, aliphatic and aromatic radicals, R<sub>2</sub> is selected from the class consisting of aromatic radicals, a ring carbon atom of which is directly linked to the nitrogen atom, and aliphatic radicals a carbon atom of which is directly linked to the nitrogen atom, said carbon atom being substituted by at least two hydrogen atoms, X and Y are selected from the class consisting of hydrogen, sulfo and carboxy, and Q represents the atoms necessary to complete a six-membered isocyclic ring system.

5. The composition as defined in claim 4 wherein the energetic silver image developer is present in an amount of from .5 to 4 grams per liter of solution.

WILLY A. SCHMIDT.  
ROBERT C. GUNTHER.

REFERENCES CITED

50 The following references are of record in the file of this patent:

UNITED STATES PATENTS

| Number    | Name         | Date           |
|-----------|--------------|----------------|
| 1,954,335 | Seymour      | Apr. 10, 1934  |
| 2,301,387 | Evans et al. | Nov. 10, 1942  |
| 2,414,491 | Tulagin      | Jan. 21, 1947  |
| 2,417,514 | Neumann      | Mar. 18, 1947  |
| 2,449,919 | Weissberger  | Sept. 21, 1948 |